

## UNITED STATES PATENT OFFICE

2,515,015

LUBRICATING OIL COMPOSITION CONTAIN-  
ING POUR POINT DEPRESSANTEugene Lieber, Chicago, Ill., and Edward P. Cash-  
man, Bayonne, N. J., assignors to Standard Oil  
Development Company, a corporation of Dela-  
wareNo Drawing. Application June 20, 1946,  
Serial No. 678,167

12 Claims. (Cl. 252—46.7)

1

This invention relates to the preparation of a novel mineral oil composition which flows at lower temperatures than the oil base stock from which it is prepared. More particularly, the invention relates to the preparation of a lubricating oil composition containing an additive which gives the lubricant an unexpectedly low stable pour point.

It has been known for some time that pour depressors for waxy mineral lubricating oils can be made by a Friedel-Crafts condensation of long chain aliphatic compounds such as chlorinated paraffin wax with aromatic compounds such as naphthalene. Small amounts, e. g., 0.1% to 2.0%, of such pour depressors may lower the A. S. T. M. pour point of a waxy mineral lubricating oil, for example, from +30° F. down to a temperature ranging from 0° F. to as low as -35° F. or lower, depending upon the particular type of oil used, the nature and method of preparation of the pour depressor, and the concentration in which the latter is used. Although it has been found that such a pour depressor may reduce the A. S. T. M. pour point to -30° F. or more, the blend may still have a 40 or 50° higher stable pour point, of the order of +10° or +20° F., as determined by the Test "V" pour stability test, described in Oil and Gas Journal, vol. 42, No. 7, pp. 103-106 (June 24, 1943). In this test the samples of oil are subjected to a series of temperature cycles ranging from -25° F. to higher levels to simulate the rise and fall of temperature during a winter season. This means that when a blend of waxy lubricating oil containing a small amount of pour depressor is stored in the winter in a place where it is subject to the fluctuation of the normal atmospheric temperature, the repeated cycles of alternate warming and cooling will permit the oil blend to become solid at temperatures of 20° or 30° or even 50° F. higher than the A. S. T. M. pour point of such blends.

It has now been found, in accordance with the present invention, that if the above-described condensation product of a long chain aliphatic compound with an aromatic compound is modified by further reacting the same with a halide, oxyhalide or sulfohalide of phosphorus, surprisingly stable pour points are produced, and in fact the pour point can be so stabilized that solidification of the oil will not result at temperatures as low as -20° F., even though a similar oil containing the unmodified pour depressor would solidify at temperatures as high as +4° to +14° F. after subjecting the same to two or more cycles of rising and falling temperature.

The alkyl-aromatic type pour depressor may be

2

prepared by any of the large number of methods known to the art, one of the earliest of which was disclosed in U. S. Patent 1,815,922. In making such alkyl-aromatic condensation product, the aromatic compound to be used may be an aromatic hydrocarbon such as naphthalene, diphenyl, anthracene, etc. The long chain aliphatic compound is preferably a material such as paraffin wax which is chlorinated to a chlorine content of about 10 to about 20%. Alternatively, such chlorinated wax or equivalent material may be dehydrochlorinated to produce corresponding olefins and the olefins may be condensed with the aromatic compound. Other long chain aliphatic compounds may be used, preferably having more than ten aliphatic carbon atoms, such as stearic acid, stearyl chloride, octadecyl alcohol, cetyl alcohol, etc. These condensation products are preferably made by the use of a Friedel-Crafts type catalyst such as aluminum chloride, zinc chloride, anhydrous hydrogen fluoride, etc., preferably in the presence of an inert solvent such as 0.05 to 5 volumes, preferably 0.1 to 1.0 volume, of a highly refined kerosene, heavy naphtha, or tetrachlorethane, per volume of mixed reactant. The reaction is conducted at a temperature ranging from room temperature up to about 200° F., preferably from 90 to 150° F. The reaction is followed by hydrolysis of the catalyst by washing with water, alcohol, or alcoholic caustic, removal of the metal hydroxide by-product by filtration or otherwise, and distillation of the reaction product under reduced pressure at a temperature up to about 500° or 600° F. to obtain the high molecular weight condensation product as a distillation residue.

The class of phosphorus- and halogen-containing compounds which may advantageously be reacted with the above-described alkyl-aromatic type pour depressor may be defined by the formula  $P(Y)_m(X)_n$ , where Y is oxygen or sulfur, X is a halogen, preferably chlorine, m is 0 or 1, and n is 3 or 5. Either the monomeric or polymeric forms of these compounds may be used. Preferred examples of suitable compounds are phosphorus trichloride, phosphorus pentachloride, phosphorus oxychloride and phosphorus sulfochloride.

When modifying the aliphatic-aromatic condensation product in accordance with this invention it is preferred to employ from 2 to 20 parts by weight of the phosphorus compound for each 100 parts by weight of the aliphatic compound employed in the condensation reaction. The reaction of the phosphorus compound with the condensation product may advantageously be con-

ducted at approximately the same temperature at which the original condensation reaction took place, and often a somewhat lower temperature may be employed.

The reaction of the phosphorus and halogen compound with the aliphatic-aromatic condensation product may be conducted by carrying out the reaction with the finished condensation product, as obtained, for example, by the method described above; but it has been found advantageous to add the phosphorus compound directly to the reaction mixture in which the condensation reaction is taking place prior to the hydrolysis step, and then to continue the reaction process as described above, providing additional catalyst if necessary. In this manner it is necessary to hydrolyze the catalyst only once, and duplication of other finishing steps may be avoided.

The oil base stocks into which the additive described above is incorporated are preferably waxy mineral lubricating oils such as a paraffinic lubricating oil base stock or a mixed base, which may have been subjected to any one or more of the commonly used refining steps, such as distillation, solvent extraction, acid treating, clay treating, etc., as well as partial dewaxing. Such oil base stock may either be one which is within the known lubricating oil viscosity range, or it may be an oil of much lower viscosity, such as one which is used in the preparation of hydraulic oils, etc., and which may have a viscosity as low as 40 seconds Saybolt at 100° F.

In employing the pour depressant of the present invention it has been found desirable to use the product in the proportion of about 0.02% to 3% or so, preferably about 0.1% to 2.0%, based on the lubricating oil base stock.

The desirable results obtained by the use of the modified aliphatic-aromatic pour depressor of the present invention and detailed methods of preparing such product are given in the following examples, which are to be considered as illustrative only and not as limiting the scope of the invention in any way.

#### Example 1

(A) A pour depressor was produced by condensing 100 parts by weight of chloro-paraffin wax (containing 14.5% chlorine) with 13½ parts by weight of naphthalene, using 2 parts by weight of  $AlCl_3$  as the catalyst. The reaction was conducted at a temperature of about 125° F. in the presence of 25 parts of tetrachlorethane as solvent. After a reaction time of 4½ hours the catalyst was hydrolyzed by the addition of an excess of isopropyl alcohol and aqueous caustic soda, and the aluminum hydroxide produced by the hydrolysis was removed. The product was then distilled to remove the diluent and the unreacted constituent to a temperature of 600° F. with fire and steam.

(B) A condensation reaction was conducted in accordance with the details set forth in (A), except that 3 hours after the beginning of the reaction of the naphthalene with the chloro-paraffin, 6 parts by weight of  $PCl_5$  dissolved in 67 parts of tetrachlorethane was added to the reaction mixture over a period of 30 minutes. Reaction with the  $PCl_5$  took place quite vigorously. After the addition of the  $PCl_5$  the reaction was continued for an additional 30 minutes, making a total of 4 hours of reaction time. The product was purified and recovered as previously described in (A).

#### Example 2

The product obtained in Example 1(B) was tested by blending the same in a waxy lubricating oil having an initial pour point of +25° F. and testing the resulting blends to determine the A. S. T. M. pour point. The following results were obtained:

| 10 | Oil Blend                                 | A. S. T. M.<br>Pour Point,<br>°F. |
|----|-------------------------------------------|-----------------------------------|
|    | Unblended base oil.....                   | +25                               |
|    | Base oil-0.0375% product of Ex. 1(B)..... | +5                                |
|    | Base oil-0.05% product of Ex. 1(B).....   | 0                                 |
| 15 | Base oil-0.1% product of Ex. 1(B).....    | -10                               |
|    | Base oil-0.25% product of Ex. 1(B).....   | <-35                              |
|    | Base oil-0.5% product of Ex. 1(B).....    | <-35                              |
|    | Base oil-1.0% product of Ex. 1(B).....    | <-35                              |

#### Example 3

The "pour stability" properties of the products of Examples 1(A) and 1(B) were tested in accordance with Test "V," previously described in this specification, using blends containing 0.25% of each additive in a base oil which was a solvent extracted Mid-Continent lubricating oil fraction containing 3½% of a Pennsylvania bright stock and having a Saybolt viscosity at 100° F. of 148 and a viscosity at 210° F. of 42.7, and an A. S. T. M. pour point of +25° F. The results show the "solid point" according to Test "V," as measured in the second and third cycles of the test, which represent a temperature drop from +30° F. to -20° F. and from +20° F. to -20° F., the "solid point" signifying the temperature at which the oil becomes solid during the course of gradual fall in temperature. The results obtained were as follows:

| 40 | Pour Depressor               | Test V Solid Point,<br>°F. |                   |
|----|------------------------------|----------------------------|-------------------|
|    |                              | Second<br>Cycle            | Third<br>Cycle    |
| 45 | Product of Example 1(A)..... | +14                        | -19               |
|    | Product of Example 1(B)..... | -11                        | <sup>1</sup> DNBS |

<sup>1</sup> Signifies "did not become solid."

It is not intended that this invention be limited to the specific examples which have been given merely for the sake of illustration, but only by the appended claims in which it is intended to claim all novelty inherent in the invention and all modifications coming within the scope and spirit of the invention.

We claim:

1. A lubricating composition consisting essentially of a major proportion of a waxy mineral lubricating oil and a pour depressing amount of a product obtained by reacting a long chain chlorinated aliphatic compound having at least 10 carbon atoms with naphthalene in the presence of a Friedel-Crafts catalyst at a temperature of room temperature to about 200° F. and further reacting the product thus formed at about the same temperature range in the presence of a Friedel-Crafts catalyst with a phosphorus- and halogen-containing compound having the empirical formula  $P(Y)_m(X)_n$ , where X is a halogen, Y is a member of the class consisting of oxygen and sulfur, m is a number from 0 to 1, and n is an odd number from 3 to 5.
2. A composition according to claim 1 in which the phosphorus- and halogen-containing compound is a phosphorus chloride.

3. A lubricating composition consisting essentially of a major proportion of a waxy mineral lubricating oil and a pour depressing amount of a product obtained by condensing chlorinated paraffin wax with naphthalene in the presence of a Friedel-Crafts catalyst at a temperature from about 90° F. to about 150° F. and then condensing the product thus formed at about the same temperature range in the presence of a Friedel-Crafts catalyst with a phosphorus- and halogen-containing compound having the empirical formula  $P(Y)_m(X)_n$ , where X is a halogen, Y is a member of the class consisting of oxygen and sulfur, m is a number from 0 to 1, and n is an odd number from 3 to 5.

4. A composition according to claim 3 in which the phosphorus- and halogen-containing compound is a phosphorus chloride.

5. A composition according to claim 3 in which the phosphorus- and halogen-containing compound is phosphorus pentachloride.

6. A composition according to claim 3 in which the phosphorus- and halogen-containing compound is phosphorus oxychloride.

7. A lubricating composition comprising a major proportion of a waxy mineral lubricating oil and about 0.1 to about 2.0% by weight of the product obtained by condensing about 100 parts by weight of paraffin chlorinated to about 14.5% chlorine with 13.5 parts by weight of naphthalene in the presence of about 2 parts by weight of aluminum chloride at a temperature of about 125° F. and in the presence of a solvent, and further condensing the reaction mass with about 6 parts by weight of phosphorus pentachloride at about 125° F. in the presence of a Friedel-Crafts catalyst.

8. As a new composition of matter, a product obtained by reacting a long chain chlorinated aliphatic compound having at least 10 carbon atoms with naphthalene in the presence of a Friedel-Crafts catalyst at a temperature from room temperature to about 200° F. and further reacting the reaction mass at about the same temperature range in the presence of a Friedel-Crafts catalyst with a phosphorus- and halogen-containing compound having the empirical formula  $P(Y)_m(X)_n$ , where X is a halogen, Y is a member of the class consisting of oxygen and sulfur, m is a number from 0 to 1, and n is an odd number from 3 to 5.

9. As a new composition of matter, the product obtained by condensing chlorinated paraffin wax

with naphthalene in the presence of aluminum chloride at a temperature of from 90° F. to 150° F. and further condensing the reaction mass with phosphorus pentachloride at about the same temperature range in the presence of a Friedel-Crafts catalyst.

10. As a new composition of matter, a product obtained by condensing about 100 parts by weight of paraffin chlorinated to about 14.5% chlorine with about 13.5 parts by weight of naphthalene in the presence of about 2 parts by weight of aluminum chloride at a temperature of about 125° F. and in the presence of a solvent, and further condensing the product thus formed with about 6 parts by weight of phosphorus pentachloride at about 125° F. in the presence of a Friedel-Crafts catalyst.

11. A method of preparing a composition suitable for use as a pour depressing agent for mineral oils which comprises condensing chlorinated paraffin wax containing about 10% to about 20% of chlorine with naphthalene in the presence of a Friedel-Crafts catalyst at about 90° F. to about 150° F. and further condensing the reaction mass in the presence of a Friedel-Crafts catalyst with phosphorus pentachloride at a temperature at about 90° F. to about 150° F.

12. A method of preparing a composition suitable for use as a pour depressing agent for mineral oils which comprises condensing about 100 parts by weight of paraffin chlorinated to a chlorine content of about 14.5% by weight with about 13.5 parts by weight of naphthalene in the presence of about 2 parts by weight of aluminum chloride at a temperature of about 125° F. and in the presence of a solvent, and further condensing the reaction mass with about 6 parts by weight of phosphorus pentachloride at about 125° F. in the presence of aluminum chloride.

40 EUGENE LIEBER.  
EDWARD P. CASHMAN.

#### REFERENCES CITED

The following references are of record in the file of this patent:

#### UNITED STATES PATENTS

| Number    | Name     | Date          |
|-----------|----------|---------------|
| 1,815,022 | Davis    | July 14, 1931 |
| 2,190,715 | Jolly    | Feb. 20, 1940 |
| 2,242,260 | Prutton  | May 20, 1941  |
| 2,246,059 | Moran    | June 17, 1941 |
| 2,316,086 | MacLaren | Apr. 6, 1943  |